

# UNITED STATES PATENT OFFICE.

DAVID JULIAN BLOCK, OF CHICAGO, ILLINOIS, ASSIGNOR TO SUNBEAM CHEMICAL COMPANY, OF CHICAGO, ILLINOIS, A CORPORATION OF ILLINOIS, AND CHARLES C. HUFFMAN, OF CHICAGO, ILLINOIS.

## DYE-SOAP AND MORDANT.

1,361,811.

Specification of Letters Patent. Patented Dec. 14, 1920.

No Drawing.

Application filed April 21, 1919. Serial No. 291,715.

To all whom it may concern:

Be it known that I, DAVID JULIAN BLOCK, a citizen of the United States, and resident of Chicago, in the county of Cook and State 5 of Illinois, have discovered a certain new and useful Dye-Soap and Mordant, of which the following is a specification.

My invention relates to dye soaps and particularly to a novel combination of a dye 10 soap and mordant.

One of the principal objects of the invention is to provide a composition in which a greater range of dye may be employed in order to secure equally satisfactory results.

15 In the making of a dye soap it has been found that in order to produce a universal dye soap only a certain limited number of dyes may be used. The difficulty has been in causing the dyes of other than a certain limited number to adhere to the fabrics without the use of a mordant.

20 The present invention contemplates the addition of the mordant to the material and to mechanically mix the same therewith. 25 This is not generally practical where the dye soap is marketed in cake form for the reason that the mordant is likely to cause precipitation of the dye or oxidization or alteration of the dye stuff. I have found, 30 however, that by flaking or otherwise finely dividing the product the mordant added thereto will not injuriously affect the substance and dye stuffs may be employed which were not heretofore considered practical for 35 use in dye soaps.

35 By the word "mordant" as used herein I refer to any substance which may be used in connection with coloring matter, either as a preliminary treatment of the fabric prior to 40 the application of the dye, or color; or any after treatment intended to improve, or otherwise alter, the tone, shade, tint, evenness or uniformity of the dyeing; its fastness to light, heat, washing, topping, perspiration, 45 or chemical action; or tending to affect the solubility, or the equalizing properties of the dye.

45 In making a dye soap in accordance with my invention the material may be prepared 50 in the usual manner by suitably mixing a vegetable oil or other saponifiable substance with the necessary quantity of sodium hydroxid or other saponifying agent, to this may be added the dye stuff in solution. If

the mordant is to be actually combined with 55 the soap mass it will be added thereto in the crutcher, after which the material is immediately flaked or otherwise finely divided in order to assure solubility. The reason why the mordant does not affect the 60 dye stuff when the material is in the form of flakes is not entirely understood but it is believed to be for the reason that the flaking of the material results in the dissipation of substantially all the uncombined water and 65 there is, therefore, nothing with which the mordant can combine in solution. This theory may, however, be incorrect and I do not wish to advance it as a statement of fact.

70 In other instances the mordant will itself be flaked or finely divided and will be mechanically mixed with the soap flakes in the package which goes to the consumer.

75 As an example of the practical application of my invention I produce various shades of yellow, tan, and brown by adding to soap flakes containing as a dye, the sodium salt of diphenyldiazobi-salicylic acid (chrysamin "G") a mordant flake containing about 20% 80 Glauber's salt, and 1% soda ash. These may be directly combined with the soap flake during the process of saponification, or may be added after the soap is formed by crutching or mechanically working the salts into 85 the soap. The foregoing proportions are productive of light shades; for darker colors I double the quantity of mordant material added; this treatment is productive of brilliant yellows. For tans I use the same dye 90 flake and mordant flake, but add to this mixture a flake containing in mechanical admixture, a weight of copper sulfate equivalent to the weight of dye used.

95 As a practical example of after treatment I add to dye flakes containing the sodium salt of dimethoxy-diphenyldiazo-naphthol-disulfonic-azo-di-metatoluenediamin (direct blue black) as a dye, a soap flake carrying in mechanical admixture about 2% para formaldehyde and an equivalent weight of calcium chlorid, mechanically worked into the carefully dried soap in the crutcher. This product is considerably faster to washing than the similar, untreated dye.

100 105 As further brief examples of my invention I add tannin to the mordant flake used in connection with the hydrochlorid of

benzene-azo-meta-phenylene-diamin (chrysoidin) which makes the dye alike applicable to silk, wool, or cotton. I add soda ash to the mordant flake for use with the soda salt 5 of ditolyldiazo - dinaphthionic acid (benzopurpurin 4 B) to secure fast reds on cotton; tannin and tartar emetic to the zinc double chlorid of tetramethyl - di - paraamido - tri-phenyl-carbinol (malachite green) to render 10 the dye universally applicable to silk, wool, jute, leather and cotton.

It will be understood that the product herein claimed may be produced by the use of materials other than those herein specified and may be marketed in a condition other than the particular condition specified. Many mordants other than those specified 15

and many dyes different from those mentioned may be employed with satisfactory results and I do not wish to be limited other 20 than as indicated in the appended claims.

I claim:

1. A dye soap in the form of flakes and a mordant mixed with the flakes, substantially as described.
2. A dye soap in the form of particles and a mordant in substantially the same form combined and mechanically mixed therewith, substantially as described.

Signed at Chicago, Illinois, this 14th day 30 of April, 1919.

DAVID JULIAN BLOCK.

Witness:

T. D. BUTLER.